

## UNITED STATES PATENT OFFICE

WILLIAM LINDSAY McPHERSON, OF THE UNITED STATES ARMY, DOVER, NEW JERSEY

## EXPLOSIVE COMPOSITION

No Drawing.

Application filed April 16, 1929. Serial No. 355,652.

(GRANTED UNDER THE ACT OF MARCH 3, 1883, AS AMENDED APRIL 30, 1928; 370 O. G. 757)

The invention described herein may be manufactured and used by or for the Government for governmental purposes, without the payment to me of any royalty thereon.

3 The subject matter of this invention is an explosive composition.

The choice of ingredients for explosive compositions depends upon their favorable behavior, the availability of supply and the 10 cost of production. At the present time the development of certain domestic industries has produced as a by-product a large supply of furfural from which can be produced derivatives of furane. While this supply of 15 furfural provides a ready source from which nitro derivatives of furane may be secured, it is not a sole source of such supply and this invention is intended to cover such derivatives from whatever sources obtained.

20 I have discovered that the nitro derivatives of furane are explosive, acting similar to their analogues in the benzene series. Dinitro-furane, for example, explodes on impact of a 2-kilogram weight. This property is 25 also characteristic of the substance when combined with other ingredients. The following are examples of such explosive mixtures.

1. Nitro compounds of furane mixed with inorganic salts, such as the nitrates and chlorates of ammonium, potassium and sodium.

2. Nitro compounds of furane mixed with alkyl and aromatic compounds, such as nitro-glycerine, glycol dinitrate, diethylene glycol dinitrate, nitro-cellulose, nitro starch, the nitro sugars, the nitro benzenes, the nitro naphthalenes, the nitro furanes, the nitro phenols, the nitro cresols, etc.

3. Nitro compounds of furane mixed with nitro-cellulose, either with or without other ingredients. In this case the former compounds act as plasticizers in addition to increasing the potential of the mixture.

4. Nitro compounds of furane mixed with inert materials, such as wood flour, starch, cereal flours, kieselguhr, etc.

The nitro compounds of furane can also be used as a coating for sporting and military smokeless powders for the purpose of obtaining better ballistics.

50 Dinitro-furane may be prepared by nitra-

tion of furoic acid and upon recrystallization gives a melting point of 101.7° C. indicating high degree of purity. This material had the following properties in comparison with TNT.

55

|                            | Dinitro-furane                        | TNT                                   |    |
|----------------------------|---------------------------------------|---------------------------------------|----|
| Explosion temperature.     | 275° C.                               | 438° C.                               |    |
| Drop test, 2 k. g. hammer. | 12 inches.                            | 15 inches.                            | 60 |
| Sensitivity to detonation. | 0.19 grams mercury fulminate.         | 0.24 grams mercury fulminate.         |    |
| Brisance.                  | 29.8 grams sand crushed in sand test. | 33.0 grams sand crushed in sand test. |    |
| Loading density.           | 1.48                                  | 1.35                                  | 65 |

I claim:

1. A new explosive embodying nitro derivatives of furane.

2. A new explosive embodying dinitro furane.

3. A nitrocellulose smokeless powder, the grains of which are coated with a nitro derivative of furane.

4. A plastic composition including a nitrocellulose explosive colloided with a nitro derivative of furane.

5. A composition including an explosive and an explosive nitro derivative of furane.

6. An explosive composition including an inert ingredient and an explosive nitro derivative of furane.

WILLIAM LINDSAY McPHERSON.

85

90

95